

## UNITED STATES PATENT OFFICE

2,398,649

## TREATMENT OF WOOD

Hamline Monroe Kvalnes, Wilmington, Del., assignor to E. I. du Pont de Nemours & Company, Wilmington, Del., a corporation of Delaware

No Drawing. Application March 10, 1943,  
Serial No. 478,666

5 Claims. (Cl. 117—148)

This invention relates to the treatment of wood, and more particularly to a method for inhibiting dimensional changes therein induced by moisture and exposure.

It is an object of this invention to treat wood in order to inhibit dimensional changes therein induced by moisture and exposure. Another object is to provide a wood treatment composition which is of low cost and high activity in its ability to prevent or inhibit dimensional changes in wood. Another object is to provide a simple, stable wood-treating solution which is easy to handle and which does not yield any substantial amount of precipitate during use. Other objects will be apparent hereinafter.

These objects are accomplished in accordance with this invention which provides a process for inhibiting dimensional changes in wood induced by moisture and exposure by impregnating such wood with a freshly-prepared, relatively concentrated solution of an active methylol urea compound, and then drying the wood, said compound having a composition of from 25 to 75 mole per cent of dimethylol urea and from 75 to 25 mole per cent of monomethylol urea.

It has been discovered that when wood is impregnated with freshly-prepared aqueous solutions of particular methylol urea compounds, especially sesquimethylol urea, which have been maintained in the active state as hereinafter more fully described, the wood is stabilized against dimensional changes induced by moisture and exposure after the impregnated wood is dried.

The methylol urea compounds which have been found suitable for the impregnation are methylol ureas having from 25 to 75 mole percent of dimethylol urea and from 75 to 25 mole percent of monomethylol urea. Preferably, sesquimethylol urea is employed, and has the composition corresponding to an equimolar mixture of monomethylol urea with dimethylol urea. However, the activity of sesquimethylol urea for dimensionally stabilizing wood in accordance with the present invention is so much superior to any other methylol urea, and its stability is so great, that it has been assigned the name "sesquimethylol urea" which indicates its composition to be 1½ methylol groups for each urea nucleus. By the expression "active methylol urea compounds" is meant a methylol urea within the prescribed composition limits which is freshly prepared immediately prior to its use, or which has been stored at a temperature not higher than about 60° F. for not longer than about three months. The aqueous solutions of the methylol urea com-

pound should likewise be freshly prepared, that is they should be made up immediately prior to the wood impregnation, or be no older than several days to not more than one week.

A relatively concentrated aqueous solution is employed for the wood impregnation, suitably from about 10 to 35% by weight of active methylol urea compound, and preferably within the more restricted range of from about 15 to 30% by weight of active methylol urea compound. Higher concentrations can be used up to about 40 or 45% by weight if the solution is heated, but in general such high concentrations are unnecessary.

The pH of the impregnating solution is within 15 the neutral to alkaline range, and can even be mildly acid if promptly used. A pH of 5.0 to 11.0 is operative, and preferably the pH is kept within the more restricted range of 7.0 to 9.0 for greatest stability of the solution. If desired, buffering 20 compounds can be added to the solution, but they are ordinarily not required and therefore are omitted. The impregnation of the wood is preferably carried to substantial completion, i. e. the wood is impregnated through and through.

25 Suitable woods which can be impregnated and rendered dimensionally stable in accordance with the present invention are the hard and soft woods which can be green or seasoned, exemplary varieties being maple, oak, mahogany, hickory, walnut, 30 gum and other hard woods as well as pine, willow, cypress, spruce, balsam, Douglas fir, and other soft woods.

The impregnation of the wood with the treatment solutions can be carried out by any means 35 which thoroughly saturates the interior of the wood with the solution, such as by long-term soaking in the treatment solution, or the alternate application of vacuum and pressure while the wood is immersed in the treatment solution.

40 For thin items, a simple immersion in the treatment solution for several days, say one to four days, suffices to thoroughly impregnate the wood. Desirably, the wood is presoaked in water for several days in order to thoroughly swell the wood

45 fibers and conserve subsequent treatment solution. The vacuum-pressure method of impregnation, a more rapid method for forcing the treatment solution throughout the wood, can be carried out by evacuating the wood in a closed vessel to a relatively high vacuum of, for example, 50 to 100 mm. mercury absolute, thereafter admitting treatment solution to the vessel still under vacuum, then releasing the vacuum to atmospheric pressure and if desired superimposing a pressure of several atmospheres up to 40 or 50

atmospheres and higher. The evacuation is carried out generally for five to twenty minutes and the atmospheric or higher pressure impregnation is carried out for a similar length of time. After impregnation by any of the foregoing methods, the wood is dried to a moisture content of preferably 5 to 20% by weight, either at room temperature or in a dryer heated to 125° F. to 180° F. or higher. Preferably, the drying is effected while concurrently heating the impregnated wood to a temperature of 125 to 300° F. or higher, since elevated temperatures hasten the further condensation of methylol ureas in situ in the impregnated wood.

Illustrating how the invention may be practiced, the following impregnations of wood were carried out, the results being tabulated in Table I below. Wood veneers, measuring  $\frac{1}{8}$ " x 12" x 12" in run #1 and measuring  $\frac{1}{8}$ " x 1" x 3 $\frac{1}{2}$ " in the succeeding runs, were presoaked in water for two days and then immersed in methylol urea treatment solutions of the indicated compositions and concentrations at the indicated pH's and allowed to soak for the indicated length of time. Controls were similarly treated except for the impregnation. Run Nos. 1 and 16 to 21 were carried out on Douglas fir veneers, while run Nos. 2 to 15 were carried out on sap gum veneers. The percentage reduction in dimensional change of treated wood over untreated wood, measured tangential to the annual tree growth rings, oven dry state to water saturated state of samples, is indicated in the last column of Table I. In the table, SMU means sesquimethylol urea, MMU means monomethylol urea, and DMU means dimethylol urea.

core and the two veneer sheets previously treated as above described were used as the face plies. The press was closed, subjected to a pressure of 150 lbs. per square inch for four minutes while being heated at 240° F. The press was then opened, the resulting panel and a matched untreated panel were sanded smooth, and both panels were placed outdoors on a south exposure test fence in the vertical position for one month. After exposure, the treated plywood remained light yellow in color as at the start of the test and its surfaces were smooth and free of open checks, while in contrast thereto the untreated plywood panel was reddish brown in color, the surface was very rough, and numerous open checks had formed.

In Table I, runs #1 to #8 show that active sesquimethylol urea is effective at a pH of 5 to 11 when the solution is freshly prepared, and that at a pH of 7 to 9 superior results are secured. Runs #9 to #15 duplicate runs #2 to #8 except that the treatment solution was aged for 33 days at room temperatures before being used. Heavy precipitate was present in all of these latter runs except when the pH was 8.0. Additionally, the percent reduction in dimensional change was not nearly of the same order as when fresh treatment solution of active sesquimethylol urea was employed. Runs #16 and #17 show that sesquimethylol urea is still active when stored at 0° C. for 47 days while the activity is greatly reduced when stored for as long as 212 days at 0° C. Run #19 shows the inferior results obtained with monomethylol urea and run #21 shows inferior results obtained with dimethylol urea. Run #20 is inserted as a comparison with run #21, the

Table I

| Run No. | Methylol urea used | Age and storage conditions of methylol urea used | Concentration of sol'n in per cent by weight | pH of sol'n | Age of sol'n in days | Precipitation in sol'n | Soaking period in days | Per cent reduction in dimensional change of treated wood over untreated wood |
|---------|--------------------|--------------------------------------------------|----------------------------------------------|-------------|----------------------|------------------------|------------------------|------------------------------------------------------------------------------|
| 1.      | SMU                | Fresh                                            | 20.0                                         | 7.0-9.0     | Fresh                | None                   | 2                      | (1)                                                                          |
| 2.      | SMU                | 24 days at 0° C.                                 | 18.3                                         | 5.0         | do                   | do                     | 3                      | 33.5                                                                         |
| 3.      | SMU                | do                                               | 18.3                                         | 6.0         | do                   | do                     | 3                      | 48.6                                                                         |
| 4.      | SMU                | do                                               | 18.3                                         | 7.0         | do                   | do                     | 3                      | 48.3                                                                         |
| 5.      | SMU                | do                                               | 18.3                                         | 8.0         | do                   | do                     | 3                      | 48.0                                                                         |
| 6.      | SMU                | do                                               | 18.3                                         | 9.0         | do                   | do                     | 3                      | 46.5                                                                         |
| 7.      | SMU                | do                                               | 18.3                                         | 10.0        | do                   | do                     | 3                      | 42.6                                                                         |
| 8.      | SMU                | do                                               | 18.3                                         | 11.0        | do                   | do                     | 3                      | 41.0                                                                         |
| 9.      | SMU                | do                                               | 18.3                                         | 11.0        | 33 days              | Present                | 3                      | 21.6                                                                         |
| 10.     | SMU                | do                                               | 18.3                                         | 10.0        | do                   | do                     | 3                      | 31.9                                                                         |
| 11.     | SMU                | do                                               | 18.3                                         | 9.0         | do                   | do                     | 3                      | 34.0                                                                         |
| 12.     | SMU                | do                                               | 18.3                                         | 8.0         | do                   | None                   | 3                      | 40.1                                                                         |
| 13.     | SMU                | do                                               | 18.3                                         | 7.0         | do                   | Present                | 3                      | 35.3                                                                         |
| 14.     | SMU                | do                                               | 18.3                                         | 6.0         | do                   | do                     | 3                      | 28.3                                                                         |
| 15.     | SMU                | do                                               | 18.3                                         | 5.0         | do                   | do                     | 3                      | 15.1                                                                         |
| 16.     | SMU                | 47 days at 0° C.                                 | 18.3                                         | 7.8         | Fresh                | None                   | 1                      | 47.0                                                                         |
| 17.     | SMU                | 47 days at 0° C.                                 | 18.3                                         | 7.8         | do                   | do                     | 3                      | 49.3                                                                         |
| 18.     | SMU                | 212 days at 0° C.                                | 20.0                                         | 7.8         | do                   | do                     | 1                      | 31.5                                                                         |
| 19.     | MMU                | Fresh                                            | 35.0                                         | 6.8-9.0     | do                   | do                     | 3                      | 16.2                                                                         |
| 20.     | SMU                | do                                               | 9.7                                          | 6.8-9.0     | do                   | do                     | 3                      | 25.4                                                                         |
| 21.     | DMU                | do                                               | 10.0                                         | 6.8-9.0     | do                   | do                     | 3                      | 13.2                                                                         |

<sup>1</sup> See note A (exposure test).

**Note A.**—The impregnated veneers sheet of run #1 were dried at 110° F. and 50% relative humidity for two days and used to prepare dimensionally stable plywood by the following procedure. An untreated  $\frac{1}{8}$ " x 12" x 12" sheet of Douglas fir veneer was used as the core and two veneer sheets treated as in run #1 were used as the face plies to prepare  $\frac{1}{8}$ " Douglas fir plywood. A conventional plywood press adapted to be heated was employed, and a commercial urea-formaldehyde hot press adhesive was used at the rate of 20 lbs. per thousand square feet of single glue line. The glue was coated on both sides of the

concentration of solution being about the same.

From the foregoing, it is apparent that freshly prepared solutions of active methylol ureas corresponding approximately to sesquimethylol urea in composition, are greatly superior to other methylol ureas.

The dimensionally stabilized wood treated in accordance with the present invention can also be treated with preservatives such as fungicides, insecticides, and the like, but free urea is preferably absent. Sesquimethylol urea is preferably prepared by dissolving and reacting three moles of dimethylol urea in water with one mole of

crystalline urea. Thereafter, the solution containing sesquimethylol urea can be evaporated at low temperature to a low moisture content of less than 10% by weight and stored under refrigerated conditions until used, but should be used within about three months. Preferably, sesquimethylol or other methylol ureas should be freshly prepared and used immediately.

Various changes may be made in the detailed practice of the invention without departing from the spirit and scope thereof.

What is claimed is:

1. A process for inhibiting dimensional changes in wood induced by moisture and exposure which comprises impregnating such wood with a solution consisting substantially entirely of water and active methylolureas having a concentration of from 10 to 45% by weight, said methylolureas having from 25 to 75 mole percent of dimethylolurea and 75 to 25 mole percent of monomethylolurea, said solution having a pH of 7 to 9, and thereafter drying the resultant impregnated wood.

2. The process of claim 1 in which the said drying is effected while concurrently heating the impregnated wood to a temperature of 125° to 300° F.

3. The process of claim 1 in which the said drying is continued at a temperature of about 125° to 180° F. until the moisture content of the wood reaches about 5% to 20% by weight.

4. The process of claim 1 in which the said methylolureas have 1½ methylol groups per urea nucleus.

5. A process for inhibiting dimensional changes in wood induced by moisture and exposure which comprises preparing a solution consisting substantially entirely of water and an equimolar mixture of monomethylolurea and dimethylolurea by dissolving and reacting three moles of dimethylolurea in water with about one mole of urea, said solution having a pH of 7 to 9, and thereafter impregnating wood with the said solution and drying the resultant impregnated wood.

HAMLINE MONROE KVALNES.